

3,227,533

## CORROSION RESISTANT COMPOSITIONS

Melvin E. Gililand, Port Arthur, and James R. Zoller, Groves, Tex., and Lawrence R. Burns, Brigham City, Utah, assignors to Texaco Inc., New York, N.Y., a corporation of Delaware  
 No Drawing. Filed Aug. 31, 1961, Ser. No. 135,135  
 9 Claims. (Cl. 44—66)

This invention relates to a corrosion inhibitor and corrosion inhibited fuel compositions. More particularly it relates to a corrosion inhibitor composition and to petroleum distillate fuels having said composition incorporated therein which are haze resistant, essentially unreactive with water and of a low cloud point.

In coassigned, copending application Serial No. 860,114, filed December 17, 1959, now U.S. Patent No. 3,036,903, a paraffinic lubricating oil oxidate having a neutralization number (neut. No.) between about 55 and 80, a saponification number (sap. No.) between about 100 and 200, an unsaponifiable content less than about 55 percent, a viscosity of less than 200 Saybolt Universal seconds (SUS) at 210° F. and a pour point less than 30° F. is taught as a corrosion inhibitor in petroleum liquids such as the petroleum fuels, for example, gasoline, naphthas, kerosene and furnace oils. The preferred lube oil oxidates are listed as having a neut. No. between 60 and 70, a sap. No. between 120 and 165, an unsaponifiable content less than 55 percent, a viscosity less than 100 SUS at 210° F. and a pour point less than 10° F.

The source and manufacture of the aforescribed lube oil oxidates are described in coassigned U.S. Patent No. 2,978,472.

The lube oil oxidates, although liquid in nature, are very viscous and therefore to facilitate their introduction into petroleum distillate fuel were diluted in the past with solvent such as a petroleum naphtha having an API gravity of about 37°, a flash point of about 160° F., a boiling range of about 370–550° F. and a 50 vol. percent A.S.T.M. distillation point of about 450° F., an aromatic content of above about 14 wt. percent, and an olefin content of above about 1 wt. percent. Normally the lube oxidates comprised between about 50 and 90 wt. percent and the solvent comprises between about 10 and 50 wt. percent of the resultant corrosion inhibitor solution.

Although the aforescribed lube oil oxidate and their solvent solutions were effective corrosion inhibitors in petroleum distillate fuels, they did have the disadvantage of reacting with any water contained in the fuel to form insoluble precipitates. Furthermore, the lube oil oxidates and their previously described solvent solutions undesirably have been found to impart a haziness and a relatively high cloud point to the petroleum distillates such as gasoline and jet fuels when incorporated therein.

The insoluble oxidate-water reaction solids are deleterious in distillate in that they collect in the screens, pumps and fuel lines of distillate fuel consuming engines thereby contributing to the malfunction thereof. Further the oxidate-water solid has a tendency to occlude water in a manner to prevent its ready removal. Water in jet fuels used in the operation of high altitude aircraft is particularly disadvantageous. These fuels must be substantially water-free otherwise there is the constant hazard in high altitude flying of water collecting and freezing in the fuel lines, pumps and screens of the aircraft thereby resulting in "flame-out" of the jet engine. In addition to the foregoing a cloudy haze in a normally clear petroleum distillate fuel creates considerable consumer resistance to the product whether or not it has actual detrimental effect.

We have discovered a composition of a reduced cloud

point that acts as an outstanding corrosion inhibitor in petroleum distillate fuels and does not form hazes or insoluble precipitates therein. More particularly, these desirable properties are found in the inhibitor combination comprising (1) the paraffinic lube oil oxidate as heretofore described, (2) a polymerized fatty acid selected from the group consisting of dimers and trimers of ethylenic fatty acids of from 12 to 22 carbon atoms and mixtures thereof, and (3) a paraffinic petroleum solvent having an olefinic content between about 0 and 0.9 wt. percent, an aromatic content less than about 12 wt. percent, a boiling point between about 300 and 650° F., an API gravity of between about 40 and 60° and a viscosity (SUS) at 100° of between about 25 and 40. The solvent and polymerized fatty acid contemplated herein are believed to function in combination to repress the haze forming and water reaction tendency of the lube oil oxidate. In addition the polymerized fatty acid surprisingly has been found to substantially reduce the cloud point of said oxidate in fuels.

Desirable ingredient amounts in the foregoing oxidate composition is between about 30 and 70 wt. percent oxidate, preferably between 40 and 60 wt. percent, between about 1 and 10 wt. percent polymerized fatty acid, preferably between 3 and 7 wt. percent, and between about 25 and 70 wt. percent petroleum paraffinic solvent, preferably between 35 and 60 wt. percent.

The amount of our inhibitor composition incorporated in petroleum distillate fuels will vary depending on the corrosive conditions encountered and the intended use of the fuel, however, for most purposes advantageous amounts range from about 1 to about 100 pounds (lbs.) inhibitor/thousand barrels (M bbls.) of distillate fuel. Typical concentrations that have been found useful in preventing rusting of iron surfaces are from about 4 to 8 lbs. of inhibitor/M bbls. of distillate for pipeline protection and from about 10 to 30 lbs. of inhibitor/M bbls. of distillate for auto, aircraft and oil burner protection.

Examples of the distillate fuels contemplated herein are those petroleum distillates having a boiling point range between about 80 and 650° F. such as gasoline, kerosene, jet fuels (JP-4, JP-5), naphthas and furnace oils.

In respect to the polymerized fatty acid ingredients (dimers, trimers and mixtures thereof) contemplated herein their physical properties are set forth in varying degrees in such U.S. Patents as 2,482,761 to Goebel, 2,631,979 to McDermott, and 2,632,695 to Landis et al. It has been shown that material consisting primarily of the dimer acid can be prepared by subjecting unsaturated fatty acids to moderate steam pressures of from 80 to 300 p.s.i., at temperatures of from 260 to 360° C. for a period of about 3 to 8 hours.

Another method for preparing the dimer acids broadly comprises heating a short chain aliphatic alcohol ester of ethylenic fatty acid at about 300° C. for several hours in an inert atmosphere. The resulting dimerized ester is then separated by distillation and hydrolyzed with hydrochloric acid or its equivalent. Fatty oils have also been heated to polymerize and thereafter hydrolyzed to produce dimer acids. The first mentioned method of preparation is preferred however, owing to the fact that a large percentage of dimer acids are produced from the starting materials by the utilization of that method of production.

The trimer acid material is quite easily obtained. It can be separated as it forms along with the monomers and higher polymer acids during the preparation of dimer acids by the methods just described. In the case of the trimer acids, however, conventional methods for preparing polymer acids are preferred over the method of Goebel, U.S. Patent No. 2,482,761, wherein unsaturated acids are subjected to moderate steam pressure, at moder-

ate temperature for a few hours, since these other methods produce high percentage of trimer acid material.

The mixture of dimer and trimer acids formed in these processes are at times, for commercial reasons, separated from monomeric and higher polymeric material present as well as from each other. However, the dimer and trimer acids can be employed in the invention compositions either separately, mixed or with minor degrading amounts of monomer and higher polymer acids.

The dimer and trimer acids and mixtures thereof of the ingredients of the present invention, although preferably conjugated products of two and three of the same molecules which are the di- or polyethylenic, are also products of the combination of monoethylenic compounds and polyethylenic compounds. For instance, linoleic acid and oleic acid dimerize to become the dimer of linoleic and oleic acids. It is, however, necessary to have at least one polyethylenic compound present to form the dimer and trimer.

The fatty acids useful in accordance with this invention include ethylenic, monocarboxylic acids having from 12 to 22 carbon atoms, examples of which are as follows: 4-dodecanoic, 5,9-dimethyl-2, 8-decadienoic, myristoleic, palmitoleic, oleic, linoleic, (9,11-octadecadienoic, 10,12-octadecadienoic, 11,13-octadecadienoic) linolenic, erucic and 13,15-docosadienoic. The preferred acid is linoleic acid on the basis of availability, cost and function in the novel compositions of the invention. Good source materials from which these fatty acids can be obtained by hydrolysis are vegetable oils, such as soy bean oil, linseed oil, cotton seed oil, corn oil, castor oil, mustard seed oil and peanut oil.

Examples of the percentage composition of the polymerized fatty materials consisting essentially of a dimer acid, trimer acid or mixtures thereof which are useful in accordance with the invention are as follows:

|                                       | Wt. percent |
|---------------------------------------|-------------|
| (1) Dimer acid                        | 78          |
| Trimer and higher polymer acids       | 22          |
| (2) Dimer acid                        | 72          |
| Trimer and higher polymer acids       | 20          |
| Monomer acid                          | 8           |
| (3) Dimer acid                        | 85          |
| Trimer and higher polymer acids       | 12          |
| Monomer acid                          | 3           |
| (4) Dimer acid                        | 92          |
| Trimer and higher polymer acids       | 6           |
| Monomer acids                         | 1.5         |
| Fatty residue material                | 0.5         |
| (5) Dimer acid                        | 99.5        |
| Fatty residue material                | 0.5         |
| (6) Trimer acid                       | 53          |
| Dimer acid                            | 35          |
| Monomer acid                          | 6           |
| Higher polymer acid and fatty residue | 6           |
| (7) Trimer acid                       | 85          |
| Dimer acid                            | 6           |
| Higher polymer acid                   | 5           |
| Monomer acid                          | 4           |
| (8) Trimer acid                       | 65          |
| Dimer acid                            | 35          |
| (9) Trimer acid                       | 98          |
| Fatty residue                         | 2           |

A preferred polymerized acid material consists of about 78 wt. percent of the dimer of linoleic acid and 22 wt. percent of the trimeric and higher polymers of linoleic acid. This dimer acid material is a light colored 36 carbon unsaturated dibasic acid and has the following properties:

|                       |     |
|-----------------------|-----|
| Acid value            | 185 |
| Saponification number | 190 |
| Neut. equivalent      | 300 |

|                                     |     |
|-------------------------------------|-----|
| Color; (Gardner)                    | 9   |
| Viscosity at 25° C. (Gardner-Holdt) | 24  |
| Flash point, ° F.                   | 530 |

5 As previously stated the petroleum solvent ingredient is paraffinic hydrocarbon petroleum distillate boiling in the range of between about 300 and 650° F. More particularly it is further characterized by a gravity between about 40 and 60° API, a viscosity (SUS) of between about 25 and 40 at 100° F., an aromatic content between 0 and 12 wt. percent and an olefin content between 0 and 0.9 wt. percent with the remainder of the solvent being composed of normal and branch chain alkanes. A preferred solvent has a boiling range between about 325 and 575° F., a gravity of about 52° API, a viscosity (SUS) of about 32 at 100° F., an aromatic content of about 5 wt. percent and an olefin content of about 0 wt. percent.

The inhibitor composition of the invention has the 20 advantage of being compatible with many fuel additives whose particular function is not related to corrosion inhibiting. For example, in fuel oil distillates having a boiling point between about 300 and 650° F., sulfurized metal phenates, such as the CO<sub>2</sub> neutralized sulfurized 25 basic alkaline earth metal alkyl (C<sub>5</sub> to C<sub>24</sub>) phenolates, are often employed to prevent the formation of sludge. These phenates are described in U.S. Patent Nos. 2,360-302, 2,362,291, 2,451,345 and 2,739,051. The inhibitor 30 composition of the invention has been found to be particularly effective and compatible with the phenates in furnace oils in a weight ratio of corrosion inhibitor composition to phenate of between about 1:10 and 10:1. The 35 total oxidate-phenate combination mixture is advantageously present in furnace oils in an amount between about 5 and 100 lbs./M bbls. of furnace oil. A preferred phenate additive is a mixture of CO<sub>2</sub> neutralized sulfurized basic barium monoalkyl phenolates where the overall barium content is between about 8 and 12 wt. percent and the monoalkyl group varies from 10 to 12 carbon 40 atoms in chain length.

The following examples further illustrate the invention but are not to be taken as limiting thereof:

#### EXAMPLE I

45 This example illustrates the preparation of the corrosion inhibitor composition of the invention.

The ingredients employed in the procedure are as follows.

#### Paraffinic lube oil oxidate

|                             |      |
|-----------------------------|------|
| 50 Characteristics:         |      |
| Neut. No.                   | 73   |
| Saponification No.          | 140  |
| Unsaponifiable, wt. percent | 40   |
| Gravity, ° API              | 16   |
| Viscosity, SUS—             |      |
| At 100° F.                  | 1207 |
| At 210° F.                  | 78   |
| Pour, ° F.                  | 0    |
| Color, Lovibond 1/2" cell   | 60   |

#### Polymerized acid

|                                                               |    |
|---------------------------------------------------------------|----|
| Ingredients:                                                  |    |
| Dilinoleic acid, wt. percent                                  | 78 |
| Trilinoleic acid and higher polylinoleic acid, weight percent | 22 |

|                             |        |
|-----------------------------|--------|
| Characteristics:            |        |
| Neut. No.                   | 192    |
| Sap. No.                    | 197    |
| Unsaponifiable, wt. percent | 0.36   |
| Gravity, ° API              | 15.9   |
| Viscosity, SUS—             |        |
| At 100° F.                  | 15,591 |
| At 210° F.                  | 476    |
| Pour, ° F.                  | 5      |
| Color, Lovibond 1/2" cell   | 40     |

**5**  
**Solvent**

## Contents:

|                                 |         |
|---------------------------------|---------|
| Olefins, wt. percent            | 0       |
| Aromatics, wt. percent          | 8.9     |
| Alkanes, wt. percent            | 91.1    |
| Characteristics:                | 5       |
| Gravity, ° API                  | 52.3    |
| Flash, TCC, ° F.                | 138     |
| Refractive index                | 1.42912 |
| Vol. percent distilled at ° F.— |         |
| Initial B.P.                    | 364     |
| 10%                             | 366     |
| 50%                             | 382     |
| 90%                             | 476     |
| 100%                            | 566     |

To a steel tank 41,916 lbs. of said paraffinic lube oil oxidate and 41,916 lbs. of said solvent were added under mixing conditions. The resultant mixture was passed to a settling tank where it was stored for 60 hours at ambient temperature. At the end of the 60 hour period two layers had formed with the bottom layer comprising an insoluble precipitate and constituting 7 wt. percent of the tank contents. The precipitate was withdrawn and discarded. The upper layer was passed through a 130 ft.<sup>2</sup> Dorr-Oliver precoat filter at 6.5 gal./hr./ft.<sup>2</sup> and 100° F. using a fine diatomaceous silica, as the precoat filter. To 31,060 lbs. of the filtered oxidate solution there was added 1553 lbs. of said polymerized acid at ambient temperature and the resultant composition was mixed for a period of 7 hours by recirculating at a rate of 10 bbls./hr. The final composition contained 44 wt. percent of said oxidate, 51 wt. percent of said solvent and 5 wt. percent of said polymerized acid. Tests on the finished product found it to have a neut. No. of 32.0, a sap. No. of 57, and unsaponifiable content of 25 wt. percent, an API gravity of 36°, a flash point of 135° F., a viscosity (SUS) of 58.6 at 100° F. and 45.9 at 130° F., a Lovibond 1/2" cell color rating of 10, a pour point of -50° F. and a cloud point of -40° F.

**EXAMPLE II**

This example illustrates the outstanding haze resistant and water reaction resistant properties of the liquid oxidate compositions contemplated herein.

Two compositions were subjected to the water-reaction test. The water reaction test is described in U.S. Patent No. 2,978,472 and is a measure of the reactivity of a distillate additive to water in a concentration of 20 lbs. additive/M bbls. isoctane. Composition A is the oxidate-solvent-polymerized acid composition of the invention prepared in Example I. Composition B is identical to Composition A except the solvent employed has a distillation range from 280 to 564° F., a 50 vol. percent distillation point of 476° F., an aromatic content of 15.3 wt. percent, an olefinic content of 1.3 wt. percent and the remainder of the solvent being composed of alkanes.

The following numerical ratings were used to evaluate the reactivity of the test compositions in the water reaction test, the higher the rating the greater the reactivity.

Rating: Appearance of the test sample

- 1 \_\_\_\_\_ Clear and clean.
- 1b \_\_\_\_\_ A few bubbles around the periphery of the interface and no shreds of lace and/or foam on the interface.
- 2 \_\_\_\_\_ Shred of lace and/or foam at the interface.
- 3 \_\_\_\_\_ Lose lace and/or slight scum.
- 4 \_\_\_\_\_ Light lace and/or heavy scum.

It was found that Composition A gave the rating of 1 and Composition B gave a rating of 2 thereby demonstrating the necessity of the combination of the particular polymerized acid and solvent contemplated herein in order to prevent the reaction of the oxidate ingredient with water to form undesirable solid and water occluding products.

**6**

The above water reaction test was conducted in accordance with military specification MIL-I-25017. In order for an additive to pass this military specification in respect to jet fuels the rating should not be greater than 1b.

**EXAMPLE III**

This example illustrates the haze resistant and low cloud properties of the corrosion inhibitor combination.

Compositions A and B described in Example II and Composition C which is the same as Composition A except the polymerized acid is omitted were dissolved in a JP-4 jet fuel in an amount corresponding to 20 lbs. of composition/M bbls. fuel. The fuel containing Composition A, the inhibitor combination of the invention, was clear and had a cloud point of -40° F. In contrast the JP-4 containing comparative Compositions B and C contained a significant haze and further the cloud point of Composition C was found to be 65° F.

The foregoing cloud points were determined in accordance with ASTM Test D97.

**EXAMPLE IV**

This example illustrates the corrosion inhibiting properties of the composition of the invention prepared in Example I.

The inhibitor of the invention was employed in a modified ASTM Corrosion Test designated as D665 Procedure B. The ASTM Corrosion Test was modified to the extent that the test temperature was 100° F. and the test duration was 20 hours. The following results were obtained.

| Lbs. inhibitor/M bbls. of isoctane: | Percent rust |
|-------------------------------------|--------------|
| 0                                   | 100          |
| 9.4                                 | 5            |
| 10.4                                | 5            |
| 11.3                                | 5            |
| 12.3                                | 4            |
| 13.1                                | 3            |
| 14.1                                | 3            |
| 16.1                                | 0            |

**EXAMPLE V**

This example illustrates the compatibility of the petroleum oxidate-polymerized acid-solvent combination of the invention with other additives normally found in distillate fuels such as the metal phenate stabilizers.

The inhibitor composition prepared in Example I was combined with steam treated, CO<sub>2</sub> neutralized sulfurized barium monoalkyl (C<sub>10</sub> to C<sub>12</sub>) phenolate containing 11.4 wt. percent barium in a weight ratio of inhibitor to stabilizer of 1:3. Twenty (20) lbs. of this inhibitor-stabilizer combination were incorporated into a furnace oil having an API gravity of 35.5°, a boiling range of between 370 and 631° F., and a 50 vol. percent distillation point of 480° F. The resultant furnace oil mixture (Composition D) was subjected to a modification (3 hour test period at 90° F. utilizing distilled water) of ASTM Corrosion Test D-665 and the Accelerated Stability Test. For comparison the fuel oil (Composition E) without the inhibitor and stabilizer was also tested.

The Accelerated Stability Test consists of heating 170 mls. of test oil for 2 hours at a temperature of 275° F. while bubbling air through said oil at the rate of 3 liters/hour. At the end of the 2 hour period the test oil is cooled to room temperature within 1 hour and 150 mls. of the cooled oil is vacuum filtered through a No. 1 Whatman filter paper. A rating of from 0 to 10 for the test oil is given depending on the amount of deposit from the oil remaining on the filter paper. A rating of 0 indicates no deposit on the filter paper and therefore an oil of highest stability and a rating of 10 indicates the entire filter paper covered with a heavy black deposit and therefore an oil of lowest stability.

The test results are reported below:

| Test description                                     | Composition D | Composition E |
|------------------------------------------------------|---------------|---------------|
| Corrosion test, percent rust                         | 0             | 60            |
| Accelerated stability test,<br>filter deposit rating | 1             | 8             |

As can be seen from the above the composition of the invention, Composition D, is non-corrosive and highly stable. In comparison comparative Composition E is corrosive and unstable.

We claim:

1. A corrosion inhibitor composition for distillate fuels consisting essentially of (1) between about 30 and 70 wt. percent of a paraffinic lubricating oil liquid oxidate characterized by a neut. No. between about 55 and 80, a sap. No. between about 100 and 200, an unsaponifiable content less than about 55 wt. percent, a pour point less than 30° F. and a viscosity less than 200 SUS at 210° F., (2) between about 1 and 10 wt. percent of a polymerized fatty acid consisting essentially of a member selected from the group consisting of dimers and trimers of ethylenic fatty acid of from 12 to 22 carbons and mixtures thereof, and (3) between about 25 and 70 wt. percent a petroleum distillate solvent having an API gravity between about 40° and 60°, a boiling point between 300 and 650° F., an aromatic content between about 0 and 12 wt. percent and an olefin content of about 0 wt. percent.

2. A composition in accordance with claim 1 wherein said polymerized fatty acid consists essentially of the dimer and trimer of linoleic acid and said solvent has a boiling range between about 325 and 575° F., and an aromatic content of about 5 wt. percent.

3. A composition in accordance with claim 2 wherein said inhibitor composition comprises about 44 wt. percent of said oxidate, about 51 wt. percent of said solvent and about 5 wt. percent of said polymerized fatty acid.

4. A liquid petroleum distillate fuel containing a rust inhibiting amount of a corrosion inhibitor composition, said composition consisting essentially of (1) between about 30 and 70 wt. percent of a paraffinic lubricating oil liquid oxidate characterized by a neut. No. between about 55 and 80, a sap. No. between about 100 and 200, an unsaponifiable content less than about 55 wt. percent, a pour point less than 30° F. and a viscosity less than 200 SUS at 210° F., (2) between about 1 and 10 wt. percent of a polymerized fatty acid consisting essentially of a compound selected from the group consisting of dimers and trimers of ethylenic fatty acid of 12 to 22 carbons and mixtures thereof, and (3) between about 25 and 70 wt. percent of a petroleum distillate solvent having an API gravity between about 40° and 60°, a boiling point between 300 and 650° F., an aromatic content between about 0 and 12 wt. percent and an olefin content of about 0 wt. percent.

5. A fuel in accordance with claim 4 wherein said rust

inhibiting amount is between about 1 and 100 lbs./M bbls. of said fuel.

6. A fuel in accordance with claim 5 wherein said polymerized fatty acid consists essentially of the dimer and trimer of linoleic acid and said solvent has a boiling point range between about 325 and 575° F. and an aromatic content of about 5 wt. percent.

7. A fuel in accordance with claim 6 wherein said inhibitor composition comprises about 44 wt. percent of said oxidate, about 51 wt. percent of said solvent and about 5 wt. percent of said polymerized fatty acid.

8. A furnace oil distillate having a boiling point between about 300 and 650° F. containing an additive combination in an amount between about 5 and 100 lbs./M bbls. of said distillate, said combination consisting essentially of a stabilizer and corrosion inhibitor in a weight ratio of said stabilizer to said corrosion inhibitor of between about 1:10 and 10:1, said stabilizer consisting essentially of a sulfurized metal phenate and said inhibitor consisting essentially of (1) between about 30 and 70 wt. percent of a paraffinic lubricating oil liquid oxidate characterized by a neut. No. between about 55 and 80, a sap. No. between about 100 and 200, an unsaponifiable content less than about 55 wt. percent, a pour point less than 30° F. and a viscosity less than 200 SUS at 210° F., (2) between about 1 and 10 wt. percent of a polymerized fatty acid consisting essentially of a member selected from the group consisting of dimers and trimers of ethylenic fatty acid of from 12 to 22 carbons and mixtures thereof, and (3) between about 25 and 70 wt. percent of a petroleum distillate solvent having an API gravity between about 40° and 60°, a boiling point between 300 and 650° F., an aromatic content between about 0 and 12 wt. percent and an olefin content of about 0 wt. percent.

9. A fuel oil in accordance with claim 8 wherein said weight ratio is 3:1, wherein said stabilizer is CO<sub>2</sub> neutralized sulfurized barium monoalkyl



phenolate, wherein said polymerized fatty acid consists essentially of dimer and trimer of linoleic acid and said solvent has a boiling range between about 325 and 575° F., and an aromatic content of about 5 wt. percent.

#### References Cited by the Examiner

#### UNITED STATES PATENTS

|           |         |                 |       |          |
|-----------|---------|-----------------|-------|----------|
| 2,360,302 | 10/1944 | Etzler et al.   | ----- | 252—32.5 |
| 2,632,695 | 3/1953  | Landis et al.   | ----- | 44—66    |
| 2,739,051 | 3/1956  | Roger et al.    | ----- | 44—76    |
| 2,916,454 | 12/1959 | Bradley et al.  | ----- | 44—76    |
| 2,978,472 | 4/1961  | Kirkwood et al. | ----- | 252—55   |

DANIEL E. WYMAN, Primary Examiner.